

April 18, 1933.

A. C. FISCHER

1,903,756

EXPANSION JOINT FOR CONCRETE ROADS

Original Filed Sept. 4, 1924

Fig. 1



Fig. 2



Fig. 3



Fig. 4



Fig. 5



Fig. 6.



Fig. 7



Fig. 8



Fig. 9.



Fig. 10



INVENTOR:

Albert C. Fischer,

By Wilkinson, Harley, Gray & Knight,  
ATTORNEYS.

## UNITED STATES PATENT OFFICE

ALBERT C. FISCHER, OF CHICAGO, ILLINOIS, ASSIGNOR, BY MESNE ASSIGNMENTS, TO  
THE PHILIP CAREY MANUFACTURING COMPANY, A CORPORATION OF OHIO

## EXPANSION JOINT FOR CONCRETE ROADS

Application filed September 4, 1924, Serial No. 735,927. Renewed March 20, 1931.

Heretofore it has been customary to manufacture expansion joints by building up in alternate layers felt and asphalt mastic; also it has been customary to manufacture an expansion joint on an asphaltic mastic center and felt sides. The felt has been depended upon for a stiffening means and rigidity, causing the expansion joint to be rigid vertically and horizontally.

10 My invention relates primarily to a structure which is flexible horizontally and rigid vertically. It has been customary in rolling steel to press out the ingots between pressure rolls, elongating them into long strands.

15 Likewise asphalt in flat strips one or two inches in thickness and several inches in width, when in a plastic, rubbery condition, under the same treatment, will elongate along the lines of its length and will vary little, if any, in the width, so that a strip of asphalt, several inches thick and several feet in length when reduced in thickness to approximately one-quarter or half an inch in thickness, will elongate to three or four times the number 20 of feet in length. When a paper surfacing, saturated felt, dried felt, wood veneer and like materials are placed either in the center or on the sides and surrounded by asphalt or allowed to be exposed on the surface, is placed on a one or two inch thickness and pressed between rolls, the fibrous matter or covering being of a semi-rigid structure breaks apart when the asphalt is pressed to a thinner dimension, because the plastic 25 matter presses out and elongates and the rigid matter, due to adhesion, must therefore break transversely into narrow sections by reason of the pressure and the non-plastic condition of the fibrous material. Thus, if 30 a paper or flat sheet of any like material is placed on the side of an asphaltic body in a thin layer, the elongation process would break apart the layer because of its plastic condition, and there would appear upon the 35 length of the joint numerous strips transversely to the length which would be pressed into it or covered by other asphalt forced over it under pressure. It is this feature 40 which I claim to be new and which involves 45 a process heretofore not practiced, and which 50

would likewise preserve the fibrous material in an unpenetrated state, thus making a stiffening skeleton in the interior of the joint.

In the accompanying drawing,

Figures 1 and 2 show in perspective and in section, an asphaltic body with fibrous sheets applied to a surface or surfaces thereof and ready to be rolled to elongate the asphalt body and subdivide the fibrous matter into spaced strips.

Figures 3 and 4 illustrate, by edge and perspective views, an application of the invention in which the fibrous matter is located interiorly of the bituminous body; Figure 3 showing the condition before elongation; 65 and Figure 4 after elongation.

Figures 5 and 6 are face views showing an application of the invention similar to that involved in Figures 1 and 2; Figure 6 illustrating the condition of the fibrous material 70 after elongation of the asphaltic body.

Figure 7 shows in perspective an effect similar to that shown in Figure 6, but existing on both sides of the body.

Figure 8 illustrates one method of treating a body such as illustrated in Figure 5 to produce the effect of Figure 6; and Figure 9 shows the effect thus produced; and

Figure 10 illustrates a form of apparatus 80 for preparing the fibrous matter for application to the asphaltic body.

To better illustrate my invention I refer to the drawing, in detail Fig. 1 represents a strip of asphalt having upon its surface a scored sheet, in which *a* represents the fibrous matter and *b* the scorings along which it is desired that the fibrous matter break apart.

Fig. 2 illustrates the transverse section of this fibrous matter, in which *a* represents the fibrous material and *b* the scoring along which it is desired that the fibrous matter break.

Fig. 3 illustrates this fibrous matter with scorings placed between two layers of asphalt, 95 in which *a* represents the fibrous matter, *b* the scorings or grain, and *c* the asphaltic material. This body structure would be thicker than the desired ultimate size of the joint required and when placed between pres- 100

sure rolls it would elongate into a strip as illustrated in Fig. 4.

Fig. 4 illustrates this elongated strip, in which *a* represents the fibrous material and *cc* the asphaltic material. Some of the asphaltic material, as will be noted, has been pressed between the segments which have been broken apart, thus building in the joint skeleton of unpenetrated fibrous matter and 10 a stiffening means vertically as the break is scored transversely to the length of the joint.

Fig. 5 illustrates a wood veneer sheet showing the grain transversely of the length thereof, which when treated to the process 15 indicated would cause breakage along the grain transversely of the length thereof; *a* represents the fibrous material and *b* the scorings or markings of the fibrous material when pressed apart by having a plastic body 20 over or under it which would cause a separation of these transverse segments along the lines of the grain and cause a formation as in Fig. 6, in which *a* represents the fibrous segments broken apart, having the plastic 25 asphaltic material filling the spaces between them.

Fig. 7 illustrates how a suitable layer of fibrous matter might be inherently constructed in an asphaltic mass and built up in a tree-like formation of flaky material in thin laminae or leaves, making it a more rigid structure than illustrated in Fig. 4; *c* represents the asphaltic mass and *a* the fibrous material in double layer formation.

Fig. 8 illustrates the process of forcing a heavy bituminous strip embodying the sheet as shown in Fig. 2, in the process of going through pressure rolls, *d*, and the result shown to the right of the rolls, in which *c* represents the plastic bituminous mass and *a* the fibrous material divided in the asphaltic mass.

Fig. 9 illustrates this plastic bituminous mass after it has passed through the rolls, 45 having a final coating upon the upper surface, and how it would appear if pressed between the rolls.

Fig. 10 illustrates the process of running a veneer sheet through a series of saturating tanks over rolls as at *e*, into the tank as at *f* and gathering asphalt as at *c* in order to build up the body structure by repeated immersions and cooling and finally pressing through rolls as at *d*.

It can readily be appreciated that dividing up fibrous material of increased rigidity would increase the rigidity of the structure, and inasmuch as it would require a veneer thickness from one-sixteenth to one-eighth of an inch to give adequate strength, it would be most likely that this structure would remain unsaturated, even though it was immersed momentarily in a hot bath of molten asphalt. This would bring the invention in 60 previous applications for Letters Patent in

which various cellular matter has been shown to be incorporated in an asphaltic mass as a stiffening means. I therefore do not wish to be limited in the use of materials as a strengthening means in the body structure 70 as some very thin materials which are properly scored may be readily forced apart under pressure as outlined; and even a metal sheet, if properly scored and previously weakened along the seam, might readily be 75 broken apart and accomplish the purpose herein intended.

The bituminous material required would of necessity be blown asphalt in order to secure the rubbery condition required for expansion joint of this kind. However, other compositions might be introduced which would not affect the construction or process herein described.

I claim:

1. An expansion joint strip comprising a body of bituminous composition provided with separable thin reenforcing strips embedded in the surface of the bituminous body.

2. An expansion joint strip comprising a body of bituminous composition provided with disjoined thin reenforcing strips embedded in spaced relation in the surface of the bituminous strip.

3. An expansion joint strip comprising a body of bituminous composition provided with disjoined thin wooden strips embedded in the surface of the bituminous body.

4. An expansion joint strip comprising a body of bituminous composition provided with thin wooden strips embedded in spaced relation in the surface of the bituminous body.

5. An expansion joint strip comprising a body of bituminous composition provided with separable thin reenforcing strips embedded in both faces of the bituminous body.

6. An expansion joint strip comprising a body of bituminous composition provided with disjoined thin wooden strips embedded in both faces of the bituminous body.

7. An expansion joint strip comprising a body of bituminous composition provided with disjoined thin reenforcing strips embedded in spaced relation in both faces of the bituminous body.

8. An expansion joint strip comprising a body of bituminous compound provided with thin wooden strips embedded in spaced relation in both faces of the bituminous body.

9. A process for fabricating reenforced expansion joint strips of bituminous composition characterized by facing a bituminous base sheet with a thin reenforcing cover sheet, scoring the cover sheet transversely at intervals, and rolling the composite structure to separate the cover sheet into individ-

ual slats and embed them in the surface of the bituminous base sheet.

10. A process for fabricating reenforced expansion joint strips of bituminous composition characterized by facing a bituminous base sheet on both faces with thin reenforcing cover sheets, scoring the cover sheets transversely at intervals, and rolling the composite structure to separate the cover sheets into individual slats and embed them in the surface of the bituminous base sheet.

11. A process for fabricating reenforced expansion joint strips of bituminous composition characterized by facing a bituminous base sheet with a thin wooden cover sheet, scoring the cover sheet transversely at intervals, and rolling the composite structure to separate the cover sheet into individual slats and embed them in the surface of the bituminous base sheet.

12. A process for fabricating reenforced expansion joint strips of bituminous composition characterized by facing a bituminous base sheet on both faces with thin wooden cover sheets, scoring the cover sheets transversely at intervals, and rolling the composite structure to separate the cover sheets into individual slats and embed them in the surface of the bituminous base sheet.

13. A process for fabricating reenforced expansion joint strips of bituminous composition characterized by adhering a thin reenforcing sheet to a bituminous base to produce a laminated structure, and rolling the laminated structure to separate transversely the thin reenforcing sheet into individual slats.

The foregoing specification signed at Chicago, Illinois, this 6th day of February, 1925.

ALBERT C. FISCHER.

45

50

55

60

65